

FIP8309

XR 1,409,184

CATION OF TEXTILES &amp; FIBERS,

## 111 UNITED STATES PATENT OFFICE.

JOSEPH FRANCIS KING, OF PHILADELPHIA, PENNSYLVANIA, ASSIGNOR OF ONE-HALF TO HARRY B. HAINES, OF PHILADELPHIA, PENNSYLVANIA.

## PROCESS OF DYEING AND BLEACHING.

1,409,184.

Specification of Letters Patent. Patented Mar. 14, 1922.

No Drawing.

Application filed December 9, 1919. Serial No. 343,464.

To all whom it may concern:

Be it known that I, JOSEPH FRANCIS KING, a citizen of the United States, and a resident of the city of Philadelphia, county of Philadelphia, and State of Pennsylvania, have invented certain new and useful Improvements in Processes of Dyeing and Bleaching, of which the following is a specification.

10 My invention relates to a process of dyeing and bleaching materials, preferably plant fibers, such as cotton, linen and the like, and animal fibers, such as wool, silk and the like.

15 An object of my invention is to produce dyed and bleached goods of superior quality by a new and useful combined process of dyeing and bleaching.

Another object of my invention is to produce bleached goods having any desired color, shade or tint.

Another object of my invention is to produce dyed and bleached goods of cotton or similar texture which will have the same 25 appearance as what is commonly known as Egyptian cotton or yarn.

Another object of my invention is to produce the aforesaid goods free of foreign matter, such as specks, motes and shives, 30 usually found, for example, in raw cotton and which, when present in finished goods, affects the quality, value, and appearance thereof.

Still further objects of my invention are 35 to produce a stronger dyed and bleached goods, to remove the impurities usually present in the raw materials used to produce such goods, to save time and labor, to reduce the loss in weight of the dyed and bleached 40 goods and to improve the appearance of, as well as to produce the particular appearance and color of the goods, as desired.

In prior dyeing and bleaching processes within my knowledge, several disadvantages 45 are present among which are the great length of time necessary to complete the bleaching action, the necessity of carrying out the bleaching operation independently of and usually before the dyeing operation, 50 the large amount of labor involved, the large number of handlings and treatments necessary, the loss in weight in tensile strength of the bleached and dyed material, the great difficulty in securing uniformity of the dye- 55 ing effect and the avoidance of color or

shade striation when dyeing, the failure to obtain a dyed and bleached product having the desired grade of softness or "loft," the presence of foreign matter and impurities and the difficulty of securing permanence or 60 "fastness" of color.

In the Letters Patent of the United States, Nos. 1,321,643 and 1,321,644 I disclose certain new and useful processes for bleaching goods which might be followed by a dyeing 65 operation. By my invention herein disclosed, the dyeing operation may take place during the process of bleaching with the ultimate result of directly producing a dyed product or goods having all of the effects 70 the bleaching operation would produce combined with the desired dyed effect. Moreover, the dyeing apparently depends more upon the result arising from the chemical reaction occurring between the ingredients 75 used in my process herein disclosed than a mere pigmental impregnation, as more usually occurs in ordinary dyeing.

By the process of my invention all of the above enumerated disadvantages are sought 80 to be overcome or remedied and in carrying out my invention I find that a complete combined dyeing and bleaching action may be accomplished in approximately three quarters of an hour with a large saving of labor 85 involved and with the number of handlings and treatments of the material to be dyed and bleached reduced to a minimum. I also find that by my process there is often-times no loss in weight of the dyed and bleached 90 material and whenever any loss occurs it rarely amounts to an appreciable quantity. I further find that by my process the loss in tensile strength of the dyed and bleached material is substantially decreased and also 95 that the dyed and bleached material is of superior grade both in quality and appearance, its "loftiness" being superior to that obtained in the usual processes of bleaching and dyeing.

Moreover, by my process, impurities such as specks, motes, shives and the like which detract from the appearance and the value 100 of the finished materials or goods are eliminated with the result that the appearance 105 and quality of the material is greatly improved and the value thereof enhanced.

In carrying out my invention I may first mix a suitable quantity of the desired dye 110 with a suitable quantity of fuller's earth in

8. BLEACHING & DYEING; FLUID TREATMENT & CHEMICAL MODIFICATION OF TEXTILES & FIBERS,

111<sup>2</sup>

1,409,184

water in a suitable receptacle (of about two gallon capacity) and boil the same for a few minutes. I then place this mixture in a container containing the bleaching composition from which the mixed dyeing and bleaching materials may be fed to a boiling vat in which is contained five hundred pounds of the material or goods to be treated, immersed in water.

10 The bleaching material may be prepared by mixing together the following constituents or ingredients in substantially the proportions indicated as follows: 10 pounds of sodium peroxide; 5 pounds of sodium bi-carbonate or soda ash; 5 pounds of anhydrous sodium sulphate or Glauber's salt; 5 pounds of sodium chloride or common salt; 6 pounds of dry caustic soda or sodium hydrate, and placing this mixture in the container containing twenty gallons of water.

15 The dye mixture may be added to this mixture as above described. I may then place five hundred gallons of water in the vat, above mentioned, heat the same to boiling and place therein the goods to be treated. I then feed this dyeing and bleaching composition from the container to the vat. The goods and the materials in the vat are then continually boiled for about three quarters 20 of an hour when the dyeing and bleaching action is complete and the vat may then be drained. The goods may be permitted to cool but I have found it desirable to run cold water into the vat to cool the goods. No 25 other treatment of the goods is necessary inasmuch as all of the dyeing and bleaching action is complete at the end of the three quarter hour boiling action and moreover no rinsing is necessary. The effects produced 30 in the goods are permanent and uniformly distributed. In the above indicated composition I have found that the English clay or fuller's earth acts or appears to act in several capacities; namely, as a resister, a 35 softener, a filler, a leveler and a finisher of the goods dyed as well as to give it weight. It further appears that the mixing of the 40 dyeing material with the bleaching material permits certain reactions in the vat, whether 45 the same be chemical or otherwise, between the ingredients which effect the uniform and homogeneous coloration of the goods as 50 counter-distinguished from striation and unequal distribution of colors, shades and tints, 55 in the prior methods of dyeing.

It may be observed that in the above composition I may, if desired, use caustic potash or potassium hydrate instead of caustic soda or sodium hydrate in approximately the 60 same proportion with substantially the same result.

I have found by experiment that a dye for producing the color peculiar to Egyptian cotton may be obtained by mixing together 65 substantially 15 ounces of gray dye and sub-

stantially 5 ounces of yellow dye together with 5 pounds of fuller's earth in a receptacle containing two gallons of water, as above described.

In the process described above the function of the caustic soda in conjunction with the sodium bi-carbonate is primarily for the purpose of cleaning the material of the impurities.

If then the goods are already free of impurities it may not be necessary to give them the particular treatment required to remove such impurities and my process may omit the constituents sodium bi-carbonate and caustic soda.

From the above it may be observed that the solution is alkaline but depending upon the materials to be treated, acids may be substituted for alkalis to produce neutral or acid solutions as desired.

While I have described the manner in which the goods may be dyed and bleached, this description is intended as exemplifying rather than limiting my invention and it is to be understood that the materials used, their proportions, the order in which the steps are enumerated and the period of treatment, may be suitably varied, without departing from the spirit and scope of my invention.

Having thus described my invention what I claim as new and desire to secure by Letters Patent of the United States is:

1. A process of dyeing and bleaching consisting of dissolving sodium chloride, sodium bi-carbonate, sodium peroxide, sodium sulphate and caustic soda in water, adding a dye thereto, introducing the materials to be treated in said solution and subjecting the mass to heat.

2. The process of dyeing and bleaching consisting of placing the materials to be dyed and bleached in a solution obtained from an admixture of sodium peroxide, sodium sulphate, sodium chloride, fuller's earth and a dye.

3. The process of dyeing and bleaching consisting of placing the materials to be dyed and bleached in a solution obtained from an admixture of sodium peroxide, sodium bi-carbonate, sodium sulphate, sodium chloride, sodium hydrate, fuller's earth and a dye.

4. The process of coloring and bleaching consisting of mixing a dye and fuller's earth in hot water, dissolving sodium peroxide, sodium bi-carbonate, sodium sulphate, sodium chloride and sodium hydrate in cold water, adding the mixture to the solution, placing the materials to be treated in water, heating the same, adding the combined mixture and solution thereto while continuing to heat the same and permitting the dyed and bleached material to cool.

5. The process of coloring and bleaching

- consisting of mixing a dye and fuller's earth in hot water, dissolving sodium peroxide, sodium sulphate and sodium chloride in cold water, adding the mixture to the solution, 5 placing the materials to be treated in water, heating the same, adding the combined mixture and solution thereto while continuing to heat the same and permitting the dyed and bleached material to cool.
- 10 6. The process of dyeing and bleaching consisting in mixing a gray dye, a yellow dye and fuller's earth in water, heating the same, preparing a bleaching solution consisting of dissolving sodium peroxide, sodium 15 bi-carbonate, sodium sulphate, sodium chloride and sodium hydrate in cold water, adding thereto and mixing therewith the dye and fuller's earth mixture, placing the materials to be treated in water, heating the same, 20 adding thereto the combined dyeing mixture and bleaching solution while continuing to heat the same.
7. The process of dyeing and bleaching consisting in mixing a gray dye and yellow 25 dye and fuller's earth with water, heating the same, preparing a bleaching solution and sodium chloride in cold water, adding thereto and mixing therewith the dye and fuller's earth mixture, placing the materials to be 30 treated in water, heating the same, adding thereto the combined dyeing mixture and bleaching solution while continuing to heat the same.
8. The process of dyeing and bleaching 35 consisting in mixing a gray dye, a yellow dye and fuller's earth with water, heating the same, preparing the bleaching solution consisting of dissolving sodium peroxide, sodium bi-carbonate, sodium sulphate, so- 40 dium chloride and sodium hydrate in cold water, adding thereto and mixing therewith the dye and fuller's earth mixture, placing the materials to be treated in water, heating the same, adding thereto the combined dye- 45 ing mixture and bleaching solution while continuing to heat the same and adding cold water to the dyed and bleached material to cool the same.
9. The process of dyeing and bleaching consisting in mixing in a suitable quantity 50 of water substantially in the proportions by weight of 15 parts of gray dye, 5 parts of yellow dye, 80 parts of fuller's earth, heating the same, adding and mixing the same to and with a bleaching solution, placing the 55 materials to be treated in water, heating the same, adding the combined dyeing mixture and bleaching solution thereto while continuing to heat the same.
10. The process of dyeing and bleaching 60 consisting in mixing substantially in the proportions of 15 ounces of gray dye, 5 ounces of yellow, 5 pounds of fuller's earth in substantially two gallons of water, heating the same, preparing a bleaching solution con- 65 sisting in mixing substantially in the proportions of 5 pounds of sodium peroxide, 5 pounds of sodium bi-carbonate, 5 pounds of anhydrous sodium sulphate, 5 pounds of sodium chloride and 6 pounds of dry caustic 70 soda in substantially twenty gallons of water, mixing the dye mixture and bleaching solution together, placing the materials to be treated in substantially five hundred gallons of water, subjecting the same to a 75 boiling action, adding thereto the combined dye mixture and bleaching solution during the boiling operation and adding cold water to the dyed and bleached materials to cool the same.
11. A dyeing composition consisting of a gray dye, a yellow dye and fuller's earth.
12. A dyeing composition consisting substantially in the proportions by weight of 15 parts of gray dye, 5 parts of yellow dye 85 and 80 parts of fuller's earth.
13. A dyeing and bleaching composition obtained by the admixture of gray and yellow dyes mixed with fuller's earth, and sodium peroxide, sodium bi-carbonate, so- 90 dium sulphate, sodium chloride, sodium hydrate, and water.

In witness whereof, I have hereunto set my hand this 28th day of November 1919.

JOSEPH FRANCIS KING.